

2,896,930

METHOD OF RECOVERING URANIUM FROM  
UNDERGROUND DEPOSITJohn Roger Menke, Scarsdale, N.Y., assignor to Nuclear  
Development Corporation of America, a corporation  
of New YorkNo Drawing. Application June 10, 1954  
Serial No. 435,940

3 Claims. (Cl. 262—3)

This invention relates to the recovery of uranium, vanadium, and equivalent elements, and is particularly directed to the provision of an improved method for recovering such elements from underground deposits more efficiently and more economically than has been possible heretofore. This application is a continuation-in-part of my prior application Serial No. 202,867, filed December 27, 1950, now abandoned.

At present many of our carnotite (uranium and vanadium) mines are rather small undertakings, in part because of the irregular distribution and smallness of many of the orebodies on the Colorado Plateau. These ore deposits are usually in remote regions and frequently do not warrant great capital investment in equipment. Relatively primitive methods are therefore often used. In the better of the small mines, shallow inclined shafts lead to irregular regions of rooms and pillars mined by one to five men using breast stoping techniques. The poorer sites are one-man "gopher-holes." The ore breaks readily with simple dynamiting. In the past much valuable material has been left behind in pillars supporting weak roofs. No effort is made to monitor the concentration of dangerous gases and dusts in working areas. (Occasionally wet drilling is used to minimize dust.) Costs of mining even shallow deposits by these methods are relatively high per ton of ore handled. Only high prices and rich ores permit profitable operation of many of the deposits.

In the future, when mining operations will be forced to more difficult sites and to greater depths for ore, the safety and economy problems will become even more serious. The remoteness of the mining regions will continue to make for relatively high costs and labor turnover, indicating the need for mining methods with little need for underground man power.

My invention, in simplest terms, consists of an improved process, especially suited to mining carnotite and similar ores of the Colorado Plateau, by direct leaching of the mineral values from the underground ore deposits. The method of the invention comprises delivering a cold dilute aqueous solution of an alkali metal salt of carbonic acid, substantially at ground temperature, into direct contact with the underground uranium (or vanadium, or other equivalent) mineral deposit, recovering the solution containing dissolved uranium from the deposit, and recovering uranium from the solution.

While it has long been known that the more common uranium minerals are soluble in alkali metal carbonate solutions, it has heretofore been considered necessary for the solutions to be hot and concentrated in order to dissolve the uranium efficiently and reasonably completely. I have found, however, that efficient recovery of uranium by direct leaching in place of underground deposits can be effected using dilute solutions (containing less than 50 grams per liter of the active solvent) at a temperature no higher than the temperature of the ground in which the deposit occurs, particularly if the leaching

solution is maintained in contact with the mineral for a prolonged period of time.

It will be useful to describe first the general geologic setting for which this invention is most suited. To date most of the carnotite mine locations are at sites accidentally exposed as outcrops by deep river valleys and canyons cutting through the pregnant stratum. The mines are either shallow entries from the surface or in the sides of the exposed valley cliffs. One may expect that orebodies more subtly hidden will in the near future yield to the more powerful exploration methods in development. Geologic sections indicate that many will be overlaid with several thousand feet of overburden, thus presenting major mining problems.

The microscopic geology is also significant. It seems apparent that the carnotite minerals were deposited by circulating solutions in the sandstones soon after the sandstones were laid down. The carnotite crystals are situated on the outside surfaces of the sand grains and in the interstices of the generally porous structure. This circumstance has led, for instance, to some successful work in differential grinding techniques for concentrating the ores. The permeability of the sandstone varies rather widely, ranging from that typical of coarse building sand to that of rather well-compacted quartzite, compacted, no doubt, after deposition of the carnotite. The average material is porous and is readily permeable to circulating fluids.

Uranium in its geologic occurrences is either in the plus four or plus six valence state. In the sedimentary geology with which we are concerned at present it is almost always in the plus six state as the combined uranyl ion,  $UO_2^{++}$ . It may be brought into aqueous solution by both acid and alkali solvents.

In order to increase the solubility of uranium in the cold leach solution which is employed in accordance with the invention, it is useful to incorporate complexing agents capable of forming little-ionized complexes with uranium-bearing ions. Among the complexing agents which can be used effectively for this purpose are substances which yield oxalate, salicylate, malate, maleate, tartrate, phosphate, acetate, lactate, pyruvate, glycetyl phosphate, proteinate, acetylacetone, sulfate, fluoride, ammonium mercapto acetate (thioglycolate), thenoyltri-fluoroacetone, and sulfo-salicylate ions. These may function by forming complex ions with uranium, from which the uranium shows little tendency to dissociate, or they may function by forming soluble salts which remain relatively unionized in solution. In either event, the complexing agents reduce the amount of solvent required to extract the uranium efficiently from the underground mineral and to produce leach solutions containing a reasonably high concentration of uranium. In addition to the substances mentioned above, sucrose and formaldehyde have been found useful as complexing agents.

When, as quite often occurs, the uranium mineral is found in a deposit which is associated with a carbonate or other acid-consuming gangue, the invention contemplates using an alkaline leach solution comprising an aqueous solution of an alkali metal carbonate. (However, the use of such alkaline leach solution is not confined to ores that occur in acid-consuming gangue. These alkaline leach solutions can also be used when desired to recover uranium from ores that occur in a siliceous or other acid-insoluble matrix.) By the term carbonate I include not only the normal carbonates, but also the bicarbonates. Sodium and potassium (especially the former) carbonates and bicarbonates are the substances preferably employed in making up the alkaline leach solutions, although ammonium carbonate can be used with success, and for purposes of this specification, I include the ammonium salts in the term "alkali metal" carbonate.

The carbonate leach solution used in accordance with the invention contains in general less than 50 grams per liter of dissolved carbonates, and is prepared and used cold (i.e. at substantially atmospheric temperature or at the temperature of the underground deposit).

Uranium appears to dissolve in carbonate leach solutions largely with the formation of a soluble but little-ionized anionic uranyl carbonate complex. These uranium carbonate complexes reach equilibrium slowly, and therefore it is desirable for the solution to remain in contact with the underground uranium deposit for a prolonged period of time, in order to assure efficient extraction of uranium from the deposit and the formation of reasonably concentrated leach solutions.

While dissolution of uranium in carbonate leach solutions appears to involve formation of a little-ionized complex with the carbonate ion itself, it is possible nonetheless to use other complexing agents, as set forth above, in leach solutions employing an alkali metal carbonate as the active solvent. Substances yielding citrate ions in the leach solution are especially advantageous complexing agents to employ when an alkali metal carbonate is the active solvent, but other complexing agents as listed above may be employed if desired.

To facilitate dissolution of uranium from the deposit, and especially in operating on deposits wherein the fluid flow may be well controlled with relatively small losses of solvent, it is advantageous to incorporate an oxidizing agent such as hydrogen peroxide in the leach solution. The oxidizing agent assures conversion of uranium occurring in the deposit in lower valence states to the hexavalent form in which it is most effectively dissolved by the leach solution.

The leach solution is introduced into contact with the underground deposit and is recovered therefrom by any convenient arrangement. For example, an array of drill holes may be driven into the deposit from the surface of the ground, and the solvent may be delivered through one or more of these drill holes and then pumped to the surface again through others. Other procedures heretofore proposed for conducting leach solutions to and from underground deposits in carrying out leaching-in-place operations may also be employed.

Uranium is recovered from the leach solution in any convenient manner. It may for example be precipitated as sodium diuranate ( $Na_2U_2O_7$ ) for alkali metal carbonate solutions by the addition of caustic soda. It may be recovered as uranyl nitrate by extracting the leach solution with dimethyl ether after adding a nitrate thereto, and then distilling off the ether. Similarly, many other organic liquids are known and can be used for extracting the uranyl nitrate (and other uranium compounds) from the leach solution. If desired, the uranium may be precipitated by treatment of the leach solution with caustic soda and the precipitated sodium diuranate may be further purified by dissolving it in nitric acid and separating it from impurities by solvent extraction with ether or other organic compound. Recovery of the uranium, either directly from the leach solution, or from an organic solvent into which it has been incorporated by solvent extraction, may be effected using an ion exchange resin.

The above indicated methods for recovering uranium from the leach solution are no more than illustrative of a wide variety of available procedures for accomplishing this result. The invention is not concerned especially with the provision of any particular method for separating the uranium from the recovered leach solution. Any convenient or desirable method may be employed for this purpose.

A particular feature of the method of this invention resides in the safety with which it can be employed. It involves minimum exposure of operating personnel to radiation, and it avoids the need for exposure of mining personnel to hazardous dusts and gases.

I claim:

1. The method of recovering uranium from an underground deposit of a uranium mineral dispersed in an acid-consuming gangue which comprises delivering a cold aqueous solution containing less than 50 grams per liter of an alkali metal carbonate into direct contact with the underground deposit in situ, the temperature of said solution being substantially the same as the temperature of the deposit, maintaining the solution in contact with the uranium-bearing deposit for a prolonged period of time, then recovering the solution from the deposit, and recovering uranium from the solution.

2. The method according to claim 1, in which the solution includes an oxidizing agent.

3. The method according to claim 1, in which the solution contains a complexing agent capable of forming little-ionized complexes with uranium-bearing ions.

#### References Cited in the file of this patent

#### UNITED STATES PATENTS

|    |           |              |                |
|----|-----------|--------------|----------------|
| 35 | 565,342   | Frasch       | Aug. 4, 1896   |
|    | 1,001,480 | Ulzer et al. | Aug. 22, 1911  |
|    | 1,050,796 | Bleecker     | Jan. 21, 1913  |
|    | 1,649,385 | Blumenberg   | Nov. 15, 1927  |
|    | 1,690,446 | Grant et al. | Nov. 6, 1928   |
| 40 | 1,999,807 | Gibbs        | Apr. 30, 1935  |
|    | 2,172,683 | Reed         | Sept. 12, 1939 |
|    | 2,173,523 | Nye et al.   | Sept. 19, 1939 |
|    | 2,180,692 | Potter       | Nov. 21, 1939  |
|    | 2,388,009 | Pike         | Oct. 30, 1945  |
| 45 | 2,563,623 | Scott        | Aug. 7, 1951   |
|    | 2,630,369 | Burwell      | Mar. 3, 1953   |

#### FOREIGN PATENTS

|         |               |                |
|---------|---------------|----------------|
| 296,813 | Great Britain | Sept. 10, 1928 |
|---------|---------------|----------------|

#### OTHER REFERENCES

Handbook of Nonferrous Metallurgy, Recovery of Metals, by Liddell, pages 621, 641, published 1945, by McGraw-Hill Book Co., Inc., N.Y.

55 The Canadian Mining & Metallurgical Bulletin for October, 1953, Montreal, vol. 46, issue 498, pages 634-644.

56 Mining Engineer's Handbook, by Peele, 3rd Ed., vol. II, pp. 31-13, see "Differential Reagents," published by John Wiley & Sons, Inc., N.Y.